

## UNITED STATES PATENT OFFICE

2,340,385

## LAPPING TOOL

Foster F. Hillix, Lakewood, Ohio, assignor to The  
American Steel and Wire Company of New  
Jersey, a corporation of New Jersey

No Drawing. Application August 15, 1942,  
Serial No. 454,994

2 Claims. (Cl. 51—309)

This invention relates to lapping tools and the like, and more particularly to "finishing" laps for finishing and polishing hard metal objects such as metal-working rolls and the like.

It is a prime object of my invention to provide such a tool having the characteristics of being friable while having sufficient strength to prevent a body or block thereof from breaking up in service, and being further characterized by the capacity to erode away evenly and at a sufficient rate to properly distribute and apply an abrasive grain over the surface of the work being lapped.

I have discovered that lead and mercury compositions or alloys possess the aforesaid characteristics to a high degree, and that a lap molded therefrom affords a speedy and efficient tool in practice. In experimenting with said composition, I have found that the mercury content thereof should preferably not be less than about 28% by weight, and that the action of a lap formed therefrom is still further enhanced by increasing the mercury content up to about from 35% to 37% by weight, the balance thereof being lead.

However, in excess of 37% of mercury with the lead produces a crumbly composition which will not remain in molded form in use, and therefore is unsuitable for a lapping tool.

An excellent composition and lap thereof which has proved highly satisfactory upon hardened steel metal-working rolls embodies about 35% mercury and 65% lead, by weight. A block or lapping tool molded therefrom is sufficiently friable to provide a working face which has the desired porosity and erosion capacity to properly accommodate and apply an obvious grain for producing fine highly polished finishes.

In actual test, such a lap produced a finish upon a 10-inch x 10-inch roll in approximately thirty minutes. After use, the face of the lap showed no concentrated loading of the grain, and the surface of the roll was free of stray scratches or digs, the latter being the ruination of many an otherwise well lapped finish. The finish so produced upon the roll surface was highly polished with a desired uniformity.

10 The lap of my invention is simple and relatively inexpensive in comparison with laps employing more complicated alloys or compositions, and has the further attribute of being readily and selectively varied within the range specified 15 to produce compositions most suitable to a specific abrasive grain size or fineness.

Various changes and modifications are contemplated within the scope of the following claims.

20 I claim:

1. A finishing lap consisting of about 28% to 37% mercury by weight and the balance thereof of lead, molded into block form, characterized by being friable and having the capacity to erode 25 away evenly, while having sufficient strength to remain in molded form and to thereby apply a cutting pressure to abrasive grain.

2. A finishing lap consisting of about 35% mercury and 65% lead by weight, molded into 30 block form, characterized by being friable and having the capacity to erode away evenly, while having sufficient strength to remain in molded form and to thereby apply a cutting pressure to abrasive grain.

FOSTER F. HILLIX.